

1

2,974,103

**STABILIZATION OF WAX ACID GREASES BY MEANS OF DIPHENOL SULFIDES**

William H. Goff, Port Arthur, Tex., assignor to Texaco Inc., a corporation of Delaware

No Drawing. Filed Apr. 10, 1957, Ser. No. 651,819

5 Claims. (Cl. 252—40)

This invention relates to lubricating greases containing soaps of oxidized petroleum fractions and to a method of stabilizing such greases. More particularly, it relates to the stabilization of greases thickened with petroleum oxidate soaps by means of compounds of the class of diphenol sulfides.

Lubricating greases prepared from oxidized petroleum fractions as the saponifiable materials have the disadvantage of undergoing discoloration and surface crusting in storage, which greatly impairs their utility and marketability. Attempts which have been made heretofore to stabilize these greases against these changes by means of inhibitors of various types which are commonly employed in conventional lubricating greases have not been entirely successful, and the problem is complicated by the undesirable effects which many of the inhibitors have upon other properties of these greases, such as their texture or consistency.

It has now been found that greases prepared from oxidized petroleum fractions are very successfully inhibited against both surface crusting and discoloration during storage by means of small amounts of alkylated diphenol sulfides of the type represented by the formula



wherein the groups represented by R are lower alkyl groups containing from 1 to about 6 carbon atoms and the groups represented by R' are secondary or tertiary alkyl groups containing from 3 to about 8 carbon atoms. The groups represented by R' are preferably tertiary alkyl groups containing from 4 to 5 carbon atoms. Compounds of this class include, for example, 4,4' thio bis (3-ethyl-6-sec. amyl phenol), 4,4' thio bis (3-hexyl-6-tert. butyl-phenol) and 4,4' thio bis (6-tert. butyl meta cresol). These compounds are obtained by well known reactions, such as, for example, by reacting suitable 3,6-dialkyl phenols with sulfur dichloride.

The above compounds may be employed in petroleum oxidate greases in amounts from about 0.5 to about 5 percent by weight. They are preferably employed in amounts from about 1 to about 3 percent by weight, based on the weight of the grease.

The greases wherein these inhibitors are employed comprise essentially an oleaginous liquid thickened to a grease consistency by a metal soap of a saponifiable petroleum oxidate. The metal component of the oxidate soap may be any of the metals which are commonly employed in grease making, such as sodium, potassium, lithium, calcium, barium, magnesium, aluminum, lead and so forth. The preferred metals are those of the alkali metal and alkaline earth metal groups. The grease will ordinarily contain from about 5 to about 45 percent

2

by weight of the petroleum oxidate soap. In addition, it may contain other thickening agents such as finely divided solids or other soaps, such as those prepared from the conventional fatty acids or hydroxy fatty acids.

5 The oxidates employed in preparing the greases of this invention are oxidized petroleum fractions containing considerable proportions of saponifiable materials, such as have been employed heretofore in grease making. They are obtained by oxidizing a petroleum fraction such as a lubricating oil fraction, crude or refined wax, slack wax or petrodatum at elevated temperatures by means of an oxidizing agent such as air or oxygen, in the presence or absence of a catalyst. The preferred oxidate is a material obtained by the oxidation of a petroleum wax having a saponification number in the range from about 100 to about 500. The oxidate fraction is employed in the grease making in any convenient manner by saponification with a suitable metal compound such as oxide, hydroxide or carbonate of an alkali metal or alkaline earth metal. The saponification is conveniently carried out in situ in a minor portion of the oleaginous liquid employed in the grease.

10 The oleaginous liquid employed in these greases may be any oils suitable for use in grease making generally, such as mineral oils obtained by any of the conventional refining processes in the lubricating oil viscosity range, preferably those having viscosities from about 80 seconds Saybolt Universal at 100° F. to about 225 seconds at 210° F. For certain purposes, such as for producing 15 greases suitable for high temperature operations, various synthetic oils may be employed with advantage, such as high molecular weight ethers, esters and silicone polymer oils. Particularly suitable synthetic esters are the di-carboxylic acid esters, such as, for example, di-2-ethylhexyl sebacate, disecondary amyl sebacate and di-2-ethylhexyl azelate.

20 The following example is given for the purpose of further disclosing the invention.

40 **EXAMPLE**

A grease was prepared in accordance with this invention comprising a mineral lubricating oil thickened with about 24.7 percent by weight of a sodium-calcium soap of a wax oxidate and containing 1.5 percent by weight 45 of 4,4' thio bis (6-tertiary butyl meta cresol) as an inhibitor.

The wax oxidate employed as the saponifiable material in the grease preparation had a neutralization number of 190, a saponification number of 306 and contained 50 about 20 percent of unsaponifiables. It was obtained by oxidizing a paraffin wax obtained from a pressed distillate of SAE 10 grade. The oxidation was carried out at a temperature of 270° F., a pressure of 65 p.s.i.g. and an air rate of 20 cubic feet per hour per pound of charge, 55 in the presence of a small amount of potassium permanganate as a catalyst.

The oil base was a blend consisting of 70 percent by weight of a refined naphthene base residual oil having a Saybolt Universal viscosity at 210° F. of about 164 60 and 30 percent by weight of a refined paraffin base distillate oil having a Saybolt Universal viscosity at 100° F. of about 99.

The grease preparation was carried out by saponifying the wax oxidate with a mixture of sodium hydroxide in 65 aqueous solution and lime in suitable proportions to give a 60-40 ratio of sodium and calcium soaps, in the presence of about 1/3 of the mineral oil employed in the grease. The charge was heated to 200° F. to complete the saponification and the temperature then increased to 70 about 300° F. to dehydrate, after which the mass was allowed to cool while the remainder of the mineral oil was added gradually. The inhibitor was added to the

grease at a temperature of about 150° F. A smooth slightly stringy grease was obtained having an ASTM penetration at 77° F. of 334 unworked and 344 worked (60 strokes).

The following table shows the storage stability characteristics of this grease in comparison with those of the uninhibited grease, and also with those of the same grease containing other inhibitors of various types which are commonly employed in greases and other compositions such as rubber and paint to prevent oxidation and hardening. The storage stability test was carried out by storing the greases in one pound slip-cover cans for one year at atmospheric temperatures, and noting the change in appearance and in ASTM penetration at 77° F. which occurred.

Table I

| No.    | Inhibitor                                                                                                             | ASTM Pene., worked 60 s. |                    | Appearance                                   | 20 |
|--------|-----------------------------------------------------------------------------------------------------------------------|--------------------------|--------------------|----------------------------------------------|----|
|        |                                                                                                                       | Original                 | After 1 year       |                                              |    |
| 1..... | none.....                                                                                                             | 344                      | 360                | Very hard thin brown crust.                  |    |
| 2..... | 1.5% of phosphorus-containing hydrocarbon; commercial oxidation, polymerization and condensation inhibitor.           | 407                      | 375                | Hard brown crust, oil pockets.               | 25 |
| 3..... | 1.5% of C-25 alkyl salicylic acid.                                                                                    | 374                      | 373                | Heavy brown waxy crust. Black surface layer. |    |
| 4..... | 1.5% of phenol mixture; commercial anti-skinning agent.                                                               | 349                      | 352                |                                              | 30 |
| 5..... | 1.5% of N,N'-disubsecondary butyl-p-phenylenediamine.                                                                 | 347                      | 363                | 1/4 inch very black surface layer.           |    |
| 6..... | 1.5% of di-(2-benzothiazyl-thiomethyl) urea.                                                                          | 406                      | 398                | Dark surface.                                | 35 |
| 7..... | 1.35% of mixture of sodium salts of dithiocarbamic acid and 2-mercapto-benzothiazole; commercial oxidation inhibitor. | too soft for pene.       | too soft for pene. | No crust or discoloration.                   |    |
| 8..... | 1.5% of 4,4' thio bis (6-tert. butyl meta cresol).                                                                    | 341                      | 342                | Do.                                          | 40 |

As shown by the above data, the inhibitor of this invention prevented any crusting or discoloration of the waxate grease during storage for one year, and in addition no change in the worked penetration of this grease occurred. The other compounds, which are representative of a large number of inhibitors of different chemical types which were tested, either failed to prevent crusting or discoloration or they produced an undesirable softening of the grease on the basis of the worked penetration.

Obviously many modifications and variations of the invention as hereinbefore set forth may be made without

departing from the spirit and scope thereof and only such limitations should be imposed as are indicated in the appended claims.

I claim:

5 1. A lubricating grease which normally undergoes surface crusting and discoloration in storage consisting essentially of a mineral lubricating oil thickened to a grease consistency by about 5-45 percent by weight based on the composition of a metal soap of a saponifiable material obtained by the oxidation of a petroleum fraction wherein the said metal is chosen from the group consisting of alkali metals, alkaline earth metals and mixtures thereof, and wherein said surface crusting and discoloration are inhibited by about 0.5-5.0 percent by weight of a compound represented by the formula



wherein R is an alkyl group containing 1-6 carbon atoms and R' is selected from the group consisting of secondary and tertiary alkyl groups containing 3-8 carbon atoms.

10 2. The grease composition of claim 1 wherein R is a methyl group and R' is a tertiary alkyl group containing 4-5 carbon atoms.

30 3. The grease composition of claim 1 wherein the said saponifiable material is a wax oxidate having a saponification number in about the range 100-500.

4. The grease composition of claim 1 wherein the metal component of the said soap is chosen from the group consisting of sodium, calcium, and mixtures thereof.

35 5. A lubricating grease which normally undergoes surface crusting and discoloration in storage consisting essentially of a mineral lubricating oil thickened to a grease consistency with about 5-45 percent by weight of a mixed base sodium-calcium waxate soap and wherein said surface crusting and discoloration are inhibited by about 0.5-5 percent by weight of 4,4' thio bis (6-tertiary butyl meta cresol).

#### References Cited in the file of this patent

#### UNITED STATES PATENTS

- |           |                  |               |
|-----------|------------------|---------------|
| 2,364,338 | Beaver           | Dec. 5, 1944  |
| 2,637,695 | McKinley et al.  | May 5, 1953   |
| 2,670,383 | Beaver et al.    | Feb. 23, 1954 |
| 2,673,881 | Weissberg et al. | Mar. 30, 1954 |